

April 30, 1968

A. P. YOUNMANS

3,381,255

THIN FILM RESISTOR

Filed April 12, 1965



Fig. 1



Fig. 2

INVENTOR.

Albert P. Youmans

BY

*Flehr & Swain*

Attorneys

1

3,381,255

**THIN FILM RESISTOR**

Albert P. Youmans, Cupertino, Calif., assignor to Signetics Corporation, Sunnyvale, Calif., a corporation of California

Filed Apr. 12, 1965, Ser. No. 447,206  
6 Claims. (Cl. 338—308)

**ABSTRACT OF THE DISCLOSURE**

Thin film resistor formed of an alloy of chrome and silicon in which the silicon ranges from 55 to 73 percent.

This invention relates to a thin film resistor and material therefor particularly adapted for use in integrated circuitry.

Thin film resistors heretofore developed have, for example, utilized Nichrome, an alloy of nickel and chrome, and tantalum as resistive materials. It has been found that such thin film resistors have a distinct disadvantage in that their use is usually limited to a low ohms per square value as, for example, a maximum of 400 parts per million. Utilizing tantalum films at a substantially higher ohms per square as, for example, 1,000 to 2,000 ohms per square gives an undesirably large negative temperature coefficient of resistance (TCR). With the nickel-chromium alloy, the resistive film is very thin even at 400 ohms per square and, therefore, it is difficult to obtain much higher ohms per square values before the resistor becomes very thin and, therefore, unstable. There is, therefore, a need for a new and improved thin film resistor and material for making the same.

In general, it is an object of the present invention to provide a thin film resistor and material therefor which overcomes the above named disadvantages.

Another object of the invention is to provide a thin film resistor of the above character which has a relatively high ohms per square.

Another object of the invention is to provide a thin film resistor of the above character which is relatively stable through a range of temperatures.

Another object of the invention is to provide a thin film resistor of the above character which can be manufactured with substantially conventional techniques.

Another object of the invention is to provide a thin film resistor of the above character which is particularly adapted for use in integrated circuitry.

Another object of the invention is to provide a thin film resistor which makes it possible to obtain a substantially zero TCR.

Another object of the invention is to provide a thin film resistor of the above character which can be very thin and still be stable.

Another object of the invention is to provide a thin film resistor of the above character having excellent power handling capabilities.

Another object of the invention is to provide a thin film resistor of the above character which need not be encapsulated.

Additional objects and features of the invention will appear from the following description in which the preferred embodiment is set forth in detail in conjunction with the accompanying drawings.

Referring to the drawings:

FIGURE 1 is a top plan view showing an integrated circuit utilizing thin film resistors incorporating the present invention.

FIGURE 2 is an enlarged cross-sectional view taken along the line 2—2 of FIGURE 1, showing a thin film resistor.

In general, the thin film resistor consists of a suitable

2

body of insulating material having a surface. A thin layer of an alloy of silicon and chromium is disposed on the surface to form a resistor. Leads are secured to the thin film to make electrical contact therewith.

As shown more particularly in the drawings, the thin film resistor incorporating the present invention is particularly adapted for use in integrated circuitry as shown in FIGURE 1. The integrated circuit shown in FIGURE 1 consists of a body 11 of a suitable semiconductor material such as silicon formed with a surface 12 which, as shown in FIGURE 2, may be planar. All of the body 11, or a substantial portion of the body 11, can be doped either during crystal growth or by diffusing either an n-type or a p-type dopant through one or more surfaces of the body 11 to provide a region 13 of one conductivity as, for example, an n-type conductivity as shown in FIGURE 2.

A silicon oxide layer 16 is formed at an elevated temperature in an oxidizing atmosphere on the surface 12 of the body 11. After the oxide layer has been formed, semiconductor devices are formed in the region 13 of the body 11 by conventional techniques. Thus, by way of example, openings may be formed in the oxide layer 16 and thereafter regions of opposite conductivity are formed in the region 13 diffusing a p-type dopant through the exposed area of the surface 12 into the region 13 to form a p-type layer or region. The oxide layer can then be regrown over the opening. When only a diode is desired, holes can be formed in the oxide layer to make electrical contact with the regions of opposite polarity. When transistors are desired, an opening is also formed in the oxide layer which has been regrown and an n-type dopant is diffused through the opening into the p-type region to form an n-type within the p-type region. Thereafter, the oxide layer is regrown and holes are formed therein so that contact can be made with the different regions to provide a transistor. Thus, as shown in FIGURE 1, there is shown a Zener diode 18 and a plurality of transistors 19 made in a conventional manner.

Leads 22 and contact pads 23 are also provided to make connections to various portions of the integrated circuit.

The structure thus far described is conventional and has only been described because it forms a part of the integrated circuit in which the thin film resistors are provided.

As also shown in FIGURE 1, the integrated circuit includes thin film resistors 26 embodying the present invention. As shown particularly in FIGURE 2, the thin film resistors are formed on a suitable body of insulating material which, in the embodiment shown in FIGURE 2, consists of a layer 16 of silicon dioxide which serves as a good insulator mounted on the body 11.

The thin film resistors 26 are formed by depositing a thin layer of an alloy of chromium and silicon on the exposed surface of the silicon dioxide layer 16 in a predetermined pattern and thickness to provide a resistor of the desired characteristics. Thus, as can be seen in FIGURE 1, the resistors 26 are various sizes and have varying lengths with a plurality of convolutions or loops 26a. Additional thin film resistors 27 and 28 are provided. Means is provided for forming electrical contact with the resistive material which can be either in the form of the leads 22 or portions of other devices as, for example, transistors 19.

The thin film forming the resistors is deposited in a conventional manner as by heating the material or bombarding the same with electrons, both of which are conventional practices.

In particular, one method is to utilize vacuum evaporation with an electron beam. A chunk of the chromium-silicon alloy is placed in a water-cooled copper crucible

and the electron beam is utilized to evaporate the chromium-silicon alloy in the vacuum chamber so that it is deposited upon the substrate in the desired predetermined pattern. Alternatively, vapor deposition can be utilized which is very similar to that utilized for epitaxial growth. In this process, hydrogen reduction of silicon tetrachloride in a reaction chamber is utilized. The chromium gas or vapor, or a vapor of a chromium compound, is introduced into the system so that chromium is also deposited with the silicon to obtain the desired ratio of chromium and silicon.

By way of example, very satisfactory thin film resistors formed of an alloy of chromium silicon have been manufactured using electron bombardment having a minimum resistance of 1,000 ohms per square and having a TCR of  $0 \pm 50$  parts per million per degree Centigrade, the  $\pm 50$  parts per million corresponds to .005% per degree C. These examples are as follows:

| Substrate Temperature, °C. | Evaporation Rate        | Density | Percent Silicon | Percent Chromium | Treatment at 550° C. |
|----------------------------|-------------------------|---------|-----------------|------------------|----------------------|
| 1..... 600                 | 3 Angstroms per second. | 4.20    | 60.1            | 39.9             | Vacuum.              |
| 2..... 600                 | .....do.....            | 3.80    | 68.6            | 31.4             | Air.                 |
| 3..... 25                  | .....do.....            | 3.80    | 68.6            | 31.4             | Air.                 |

It is well known that in thin films, the resistance of the resistor changes with thickness but will not change with an increase in length as long as the thin film is kept square. The above characteristics are typical of films with a thickness range of less than 100 angstroms to over 10,000 angstroms.

Each of the factors set forth in the table above will affect the TCR, that is, the temperature coefficient of resistance of the resistor. The values set forth above show that it is possible to obtain a TCR of zero within the range of 60.1 to 68.6 percent silicon. By examining the phase diagram for chromium-silicon, it is believed that a suitable resistor can be formed having a substantially zero TCR with the silicon content of the alloy ranging from 55 to 73 percent by weight with a minimum ohms per square readily obtainable from 1,000 to over 5,000 ohms per square.

It will be noted in Examples 1 and 2 that the substrate temperature is relatively high, that is, 600° C. during the deposition of the thin film for the resistor which serves to stabilize the resistor as it is being deposited. In Example 3, the resistor is stabilized by the heat treatment after the alloy has been deposited. It is desirable to have the resistor stabilized at these high temperatures because in conventional manufacture of integrated circuitry, the devices are heat treated to 550° to alloy the aluminum which is used for the leads to the diodes 18, the transistor 19, and also to the resistors 26.

Utilizing this material, it has been found that it is possible to obtain a minimum sheet resistivity substantially above 1,000 ohms per square if desired. Thus, for example, it has been possible to obtain a sheet resistivity of 5,000 ohms per square. It has been found that such a resistor is very stable and has all the desirable characteristics pointed out above.

Although the present invention has been described as depositing the chromium-silicon alloy upon insulating material such as silicon dioxide or silicon, the material can also be readily deposited upon any other suitable insulating material such as glass or ceramic.

By way of example, in one integrated circuit of the type shown in the drawing, the resistor 27 had a value of 200 ohms and the resistor 28 had a value of 500 ohms. The largest resistor 26 had a value of 15,000 ohms.

It has been found that resistors of the present type have three very desirable characteristics or advantages. The first is a high ohms per square value or, in other

words, a high sheet resistivity. Secondly, they have a high temperature stability which includes a storage stability and a long load life under high temperature. The third important advantage is the substantially zero TCR which can be obtained.

Another distinct advantage of the present thin film resistor is that it has a relatively high power handling capability. By way of example, it has been found that under load life tests, approximately 500 milliwatts of power can be dissipated over long periods of time without adversely affecting the characteristics of the resistor. In addition, it has been found that under such load life tests, the TCR changes less than one-half of 1 percent during the first 1,000 hours, and less than .1 of 1 percent during the second 1,000 hours of the load life test. It is believed that the resistors have particularly good power handling capabilities because they are deposited upon silicon dioxide layer 16 which has good contact

with the silicon body 11 which itself is a good thermal conductor. The body 11 is normally attached or brazed to a metal header which also has power dissipating capabilities.

Although the thin film resistors incorporating the present invention have been shown in the drawings as not being encapsulated, it should be appreciated that, if desired, the thin film resistors can be encapsulated. This may be particularly desirable when cross-overs which pass over the resistors are desired. Encapsulation can be accomplished by evaporating an oxide over the resistor, either silicon dioxide or some other suitable insulating oxide.

It is apparent from the foregoing that I have provided a new and improved thin film resistor and material for use in making such thin film resistors. As pointed out above, the thin film resistors have many excellent characteristics and are particularly adaptable for use in integrated circuits. The thin film resistors can be readily utilized in devices which must operate in a temperature range of  $-55^{\circ}$  C. to  $+200^{\circ}$  C. without any difficulty and with substantially zero TCR. The chromium-silicon alloy is particularly useful as a thin film resistor because it is relatively inexpensive and has excellent characteristics when utilized for thin film resistors.

I claim:

1. In a thin film resistor, a body of insulating material having a surface, a thin layer of alloy of chrome and silicon disposed on said surface in a predetermined pattern, said alloy having a silicon content ranging from 55% to 73%, and lead means making electrical contact with the thin layer.
2. In a thin film resistor, a body of insulating material having a surface, a thin layer of an alloy of chrome and silicon disposed on the surface in which the silicon content ranges from 55 percent to 73 percent, the thin layer having a thickness ranging from under 100 angstroms to 10,000 angstroms and leads making electrical contact with the thin layer.
3. A thin film resistor as in claim 2 having a minimum of 1,000 ohms per square and having a substantial zero TCR.
4. A thin film resistor as in claim 2 having a substantially zero TCR ranging from  $-55^{\circ}$  C. to  $+200^{\circ}$  C.
5. A thin film resistor as in claim 2 having an ohms per square ranging from 500 ohms per square to over 5,000 ohms per square.

6. A resistor as in claim 2 which is stabilized to a temperature above 550° C.

References Cited

UNITED STATES PATENTS

3,310,711 3/1967 Hangstefer ----- 317—101

FOREIGN PATENTS

Ad. 10,657 3/1913 Great Britain.

OTHER REFERENCES

Hansen, M.: Constitution of Binary Alloys, McGraw-Hill, New York, 1958, pp. 560—562 relied on.

5 LARAMIE E. ASKIN, *Primary Examiner.*

E. GOLDBERG, *Assistant Examiner.*